

1

3,177,074

## COBALT BASE ALLOYS

Walter A. Luce and Glenn W. Jackson, both of Dayton, Ohio, assignors to The Duriron Company, Inc., Dayton, Ohio, a corporation of New York  
No Drawing. Filed Apr. 23, 1962, Ser. No. 189,274  
6 Claims. (Cl. 75—171)

This invention relates to cobalt base alloys and particularly to cobalt alloys which are unique in respect to corrosion resistance throughout a broad range of conditions, with particular emphasis on resistance to chemical attack in severely corrosive liquid media, while providing concomitantly therewith exceptional wear and abrasion resistance, high strength, adequate ductility and good thermal shock resistance.

A general object of the invention is the provision of alloys especially useful in bearing surfaces and similar applications involving mechanical wear, where the surfaces are unavoidably exposed to highly corrosive liquid media, for example strong mineral acid like nitric, sulfuric and hydrochloric. In order to satisfy the requirements of wear and abrasion resistance, it is essential that the alloys possess a high order of hardness, and for this invention a Brinell hardness number of approximately 300 in the alloy is considered to be a minimum which is adequate in actual service. As-cast alloys which exhibit slightly lower Brinells, say as low as about 270 but which can through appropriate treatment be hardened to the recommended level without adversely affecting other properties, are thus useful and are encompassed by the invention.

The versatility of the invention alloys in respect to corrosion resistance is outstanding. These alloys have broad corrosion resistance capabilities which are not only better than any other known cobalt alloy but are also better than most other known alloys for a similar broad spectrum of corrosive environments. Corrosion data given hereinafter for the novel alloys in some of the more common mineral acids under various conditions serves to verify their superiority. For test purposes, as presently explained, certain combinations of media, temperature and concentration have been deliberately selected to provide extremely severe conditions which produce fairly high rates of corrosion which would not generally be acceptable in commercial practice. By reducing either the temperature or concentration conditions slightly, however, acceptable resistance results can be obtained. And when the conditions are thus altered to the point where the invention alloy corrosion rates become commercially acceptable, the nearest equivalent alloys heretofore available are far inferior in one or more of these environments.

In respect to corrosion resistance, tests have established that acceptable alloys within the purview of this invention should have mean corrosion rates which generally do not exceed the following limits: 15 mils per year in 65% boiling nitric acid; 20 mils per year in 10% boiling sulfuric acid; 150 mils per year in 30%

2

boiling sulfuric; 30 mils per year in 70% sulfuric at 176° F.; 30 mils per year in 15% hydrochloric at 125° F.; and 80 mils per year in 20% hydrochloric at 100° F. The term "mean corrosion rates" as here used designates the mean rates of corrosion for five 48-hour periods, in accordance with A.S.T.M. procedure set out in Standard No. A279-44 of the Society, except that mechanical agitation of the specimen is used for more consistency. It is not to be understood that corrosion rates of as high as 150 mils per year, as in 30% boiling sulfuric acid, would be tolerated in actual practice. As a rule a maximum acceptable over-all corrosion rate is around 15 to 25 mils per year. However, as mentioned above, during testing for evaluation purposes extreme corrosion conditions were deliberately picked, and the higher rate levels given for these conditions therefore serve simply as a reference against which to measure and compare the various compositions.

20 Alloys capable of meeting the foregoing corrosion and abrasion specifications are greatly needed in industry but have not been available heretofore. Specific examples of such need are to be found particularly in chemical processing equipment, for example, chemical pump components such as shaft sleeves and impellers, and valve seats for handling corrosive fluids at various temperatures. It has long been a problem in handling such fluids to design and construct an impeller shaft for chemical pumps which is capable of serving adequately and economically. The problem has become aggravated with the need for pumps of larger capacity and higher operating speed, wherein the strength requirements have largely outstripped the capability of most materials to provide practical periods of useful life in such service. Known alloys having suitable chemical corrosion resistance are unfortunately insufficient in respect to tensile strength, hardness and ductility to withstand the type of mechanical and thermal shock to which such equipment is inevitably subjected.

25 In a centrifugal pump, for example, some of the most troublesome operating or maintenance problems occur where the shaft passes through the stuffing box. Attempt 30 has been made to use a one-piece shaft of some corrosion resistant material such as a stainless steel. Not only does this become quite expensive but the austenitic stainless steels which are suitable from the standpoint of corrosion resistance cannot be hardened beyond about 35 160 Brinell which, as above indicated, is far below the desired level, with the result that wear resistance is poor. Alternatively, the use of a stainless or carbon steel shaft fitted with a separate sleeve of "Duriron," which is a 40 vary hard material (400 to 500 Brinell) having excellent corrosive resistance, runs into problems of low tensile strength and low tolerance to thermal shock in the sleeve material. Some of the known cobalt alloys, like 45 the dental alloy "Vitallium" or "Stellite 21," have excellent hardness and wear resistance but their corrosion rates in these severely corrosive media show them to be quite insufficient for the type of service here contemplated. The mean corrosion rate of "Stellite 21" in

boiling 65% nitric acid, for example, is around 164 mils per year as compared to the desired limit of only 15 mils per year in this media as specified above, and about 8 mils per year actually achieved by the invention alloys. As a further example, the invention provides an alloy having a mean corrosion rate of 15 mils per year in a 10% nitric-3% hydrofluoric acid solution at 140° F., which is in contrast to around 75 mils per year from "Durimet 20," heretofore considered to be the best commercial alloy available for this environment. Even such exotic materials as titanium and tantalum are completely unacceptable here, and the costly nickel-base alloys are considerably worse than "Durimet 20."

We have discovered that the combined requirements of corrosion, wear and abrasion resistance, ductility, adequate tensile strength and resistance to thermal shock needed for the severe type of service contemplated herein, are possessed uniquely by certain cobalt-base alloys having carefully combined and narrowly limited ranges of components, as more fully hereinafter defined, which set these alloys quite apart from previously known materials.

The novel alloys include cobalt as the largest single component, together with carefully controlled amounts of chromium, molybdenum and copper as the other major components. Carbon is always present, of course, but in very carefully controlled low amount which will vary somewhat depending on the molybdenum-chromium content, as further defined hereinafter. Small amounts, generally appreciably less than 1%, of manganese and silicon, and in some instances nickel, iron, titanium or aluminum, may also be present for specific applications of the alloy, but the total of these must be held low and generally their inclusion in the alloy composition is undesirable if the alloy is to be used under the more drastic operating conditions. Similar small percentages of other elements used principally as deoxidants, as for example calcium, and as stabilizers, for example columbium, or hardeners, as boron for example, may also be incorporated.

The unique results of the invention, however, are obtained only within compositional limits of the major components defined below, and then only by proper balance of the components within these ranges, as more fully explained hereinafter. The limiting ranges of the alloy compositions are as follows:

|    |                           |
|----|---------------------------|
| Cr | 26.0-32.0%.               |
| Mo | 8.0-15.0%.                |
| Cu | 1.5-4.5%.                 |
| C  | From about 0.02 to 0.10%. |
| Ni | Up to 10.0% max.          |
| Fe | Up to 6.0% max.           |
| Mn | Up to 2.0% max.           |
| Si | Up to 2.0% max.           |
| Co | Balance.                  |

For shaft sleeve purposes, hardness is of paramount importance. Accordingly, a preferred alloy within the foregoing range which is particularly adapted for such use has been found to have a nominal composition of about 30% chromium, 13% molybdenum, 3.25% copper, 0.03% max. carbon, 2% nickel, 2% iron, 0.5% each of silicon and manganese, the balance (approximately 48%) being cobalt. Such alloy has a Brinell hardness number of approximately 400, a tensile strength of 60,000 p.s.i. and an elongation of about 1%. As appears more fully hereinafter, the corrosion rates of such an alloy are all well within the maximum rates previously specified. (See Alloy M in Table VII which follows.)

Where an alloy of lower hardness can be tolerated, as for pump housings and impellers, or for valve bodies, gates, seats and similar components, a somewhat more dutile composition within the foregoing over-all range is provided by the following compositional analysis: 28% chromium, 8.5% molybdenum, 3.25% copper, 0.10% max. carbon, up to 10% nickel, 2% iron, 0.5% each of manganese and silicon, the balance (approximately 48 to 58%) cobalt. Such an alloy has a hardness of 270-300 BHN, a tensile strength of approximately 75,000 p.s.i., and an elongation of 6%. Again this alloy falls within the corrosion rate test limits given. (See Alloy A in Table II.)

Such an alloy as last described, however, must in general be work hardened as by shot peening to achieve the higher hardness level. For more intricate castings, therefore, an alloy having a molybdenum-chromium content intermediate the specified limits of these elements provides a hardness of around 340 BHN, and should be used. An alloy of such intermediate hardness will have improved mechanical properties relative to the very hard (375-400 BHN) alloy, without serious reduction in wear or abrasion resistance.

An alloy having as much as 6% elongation represents substantially the maximum in respect to ductility within the invention. Although significantly less hard than others obtainable within the present teaching, it is still much superior to stainless steel. But again this maximum degree of ductility will not be realized unless all the alloying elements closely approximate the stated levels.

The shaft sleeve (very hard) alloy provides mechanical properties which are considerably improved over that of high silicon iron alloys, e.g. "Duriron," heretofore found to be the best available for service under the conditions contemplated. Although it is necessary in these shaft sleeve alloys to approach a brittle composition in order to acquire a hardness of 375 to 400 BHN, still the ductility obtained is, by comparison, a substantial improvement over that of the high silicon irons.

As the nickel content is raised, the alloy of course is softened, with consequent improvement in its ductility, and for nickel contents up to 10% the corrosion resistance is generally maintained at adequate levels for all but the very worst conditions. Here again however the level within the allowable range will be determined by the hardness and corrosion resistance requirements to be met.

Although the prior art teaches that in general substitution of tungsten for some or all of the molybdenum may be made in other alloys, this teaching definitely does not apply to the alloys of this invention, and tungsten cannot be substituted for molybdenum, nor simply added to the alloy, without seriously reducing corrosion resistance and/or increasing crack susceptibility, even at the lower molybdenum levels.

A further critical point in respect of the novel alloys is the carbon content, more particularly in the harder, i.e. shaft sleeve (375-400 BHN), composition. In this composition, carbon must be maintained at or below 0.03% maximum in order to develop the optimum corrosion resistance of which the alloy is capable. In the case of alloys of lower hardness levels, i.e. around 270-300 BHN, since these appear to respond satisfactorily to quench annealing treatments without adverse effect upon corrosion resistance, carbon contents up to 0.10% can be used but a preferred level even here is 0.07% or less.

The criticality of ranges of components of the novel alloys given above is shown by the following examples. Table I lists the compositional analyses of all of the alloys whose characteristics are listed in the subsequent tables.

Table I

| Alloy | Cr   | Mo   | Ni   | Cu   | C    | Si  | Fe   | Mn | W   | Other  |
|-------|------|------|------|------|------|-----|------|----|-----|--------|
| A     | 27.0 | 8.0  | 2.0  | 3.25 | .07  | .5  | (*)  | .5 | (*) | (*)    |
| B     | 27.0 | 18.0 | 2.0  | 3.25 | .07  | .5  | (*)  | .5 | (*) | (*)    |
| C     | 27.0 | 13.0 | 2.0  | 3.25 | .07  | .5  | (*)  | .5 | (*) | (*)    |
| D     | 35.0 | 9.0  | 2.0  | 3.25 | .07  | .5  | (*)  | .5 | (*) | (*)    |
| E     | 27.0 | 8.0  | 10.0 | 3.25 | .07  | .5  | (*)  | .5 | (*) | (*)    |
| G     | 27.0 | 8.0  | 2.0  | 4.5  | .07  | .5  | (*)  | .5 | (*) | Ti 0.5 |
| H     | 27.0 | 8.0  | 2.0  | 3.25 | .07  | .5  | (*)  | .5 | (*) | Al 1.0 |
| I     | 27.0 | 8.0  | 2.0  | 3.25 | .07  | .75 | (*)  | .5 | (*) | (*)    |
| J     | 30.0 | 9.0  | 2.0  | 3.25 | .06  | .5  | (*)  | .5 | (*) | (*)    |
| K     | 30.0 | 13.0 | 2.0  | 3.25 | .06  | .5  | (*)  | .5 | (*) | (*)    |
| L     | 28.0 | 8.5  | 2.0  | 3.25 | .06  | .5  | (*)  | .5 | (*) | (*)    |
| M     | 30.0 | 13.0 | 2.0  | 3.25 | .025 | .5  | (*)  | .5 | 3.0 | (*)    |
| N     | 28.0 | 8.0  | 2.0  | 3.25 | .025 | .5  | (*)  | .5 | (*) | (*)    |
| O     | 28.0 | 8.5  | (*)  | 3.25 | .025 | .5  | (*)  | .5 | (*) | (*)    |
| P     | 28.0 | 8.5  | 3.75 | 3.25 | .025 | .5  | (*)  | .5 | (*) | (*)    |
| Q     | 28.0 | 8.5  | 6.5  | 3.25 | .025 | .5  | (*)  | .5 | (*) | (*)    |
| R     | 28.0 | 8.5  | 2.0  | (*)  | .025 | .5  | (*)  | .5 | (*) | (*)    |
| S     | 25.0 | 8.5  | 2.0  | 1.75 | .025 | .5  | (*)  | .5 | (*) | (*)    |
| T     | 28.0 | 8.5  | 2.0  | 5.0  | .025 | .5  | (*)  | .5 | (*) | (*)    |
| U     | 23.0 | 4.0  | 2.0  | 3.25 | .025 | .5  | (*)  | .5 | 4.0 | (*)    |
| V     | 28.0 | (*)  | 2.0  | 3.25 | .025 | .5  | (*)  | .5 | 8.0 | (*)    |
| W     | 28.0 | 8.5  | 2.0  | 3.25 | .20  | .5  | (*)  | .5 | (*) | (*)    |
| X     | 28.0 | 8.5  | 2.0  | 3.25 | .10  | .5  | (*)  | .5 | (*) | (*)    |
| Y     | 27.0 | 8.0  | 2.0  | 3.25 | .05  | .5  | (*)  | .5 | (*) | (*)    |
| Z     | 23.0 | 9.0  | 2.0  | 3.25 | .05  | .5  | (*)  | .5 | (*) | (*)    |
| AA    | 27.0 | 10.0 | 2.0  | 3.25 | .05  | .5  | (*)  | .5 | (*) | (*)    |
| BB    | 28.0 | 8.5  | 2.0  | 3.25 | .06  | 1.5 | (*)  | .5 | (*) | (*)    |
| CC    | 28.0 | 8.5  | 2.0  | 3.25 | .06  | 3.0 | (*)  | .5 | (*) | (*)    |
| DD    | 28.0 | 8.5  | 2.0  | 3.25 | .06  | .5  | 6.0  | .5 | (*) | (*)    |
| EE    | 28.0 | 8.5  | 2.0  | 3.25 | .06  | .5  | 10.0 | .5 | (*) | (*)    |

\*Values considered nil since elements not intentionally added.

Balance cobalt in all cases except for incidental impurities which do not exceed 1% at most, generally less.

All heats quenched annealed from 2250° F. (air or water quench, depending on the alloy as explained in the test).

Molybdenum is one of the most critical elements in the alloy and requires close control. In most media corrosion resistance drops off quickly below and above 8% and 15%, respectively. At the high end of the molybdenum range, satisfactory compositions are obtained by proper adjustment of the elements, especially the nickel content. See Table II for the effect on corrosion resistance at various molybdenum levels.

Quite as important as corrosion resistance is the fact that the hardness changes from approximately 265 BHN at 8% molybdenum to 390 BHN at 13%. Further increase in molybdenum up to 18% increases the hardness to approximately 500 BHN. This increase in hardness is accompanied by gradual change from what, for present purposes, may be considered a ductile alloy at 8% to a very brittle material at 18%. Although at the 13% molybdenum level the alloy is not one which would conveniently be considered a ductile material, nevertheless the mechanical properties are such that it is capable of withstanding the shock and strain of mechanical stresses involved in shaft sleeve use.

tionally be considered a ductile material, nevertheless the mechanical properties are such that it is capable of withstanding the shock and strain of mechanical stresses involved in shaft sleeve use.

Table II

| Alloy | Percent Mo | Hardness |    | Mean Corrosion Rate, Mils Per Year 5-48 Hour Test Periods |                 |                 |                   |                   |                   |
|-------|------------|----------|----|-----------------------------------------------------------|-----------------|-----------------|-------------------|-------------------|-------------------|
|       |            | BHN      | Rc | 65 N,*<br>Boil.                                           | 10 S,*<br>Boil. | 30 S,*<br>Boil. | 70 S,*<br>176° F. | 15 H,*<br>125° F. | 20 H,*<br>100° F. |
| Y     | 6.0        | 245      | 24 | 8                                                         | 17              | 224             | 51                | 134               | 57                |
| A     | 8.0        | 270      | 28 | 8                                                         | 11              | 114             | 14                | Nil               | 35                |
| AA    | 10.0       | 290      | 31 | 13                                                        | 9               | 88              | 23                | Nil               | 36                |
| C     | 13.0       | 393      | 42 | 27                                                        | 6               | 111             | 19                | 4                 | 68                |
| B     | 18.0       | 472      | 50 | 175                                                       | 18              | 136             | 5                 | 172               | 100               |

\*65 N denotes 65% nitric acid. 10 S, 30 S and 70 S denote, respectively, 10%, 30% and 70% sulfuric acid. 15 H and 20 H denote 15% and 20% hydrochloric acid.

These abbreviations apply throughout the remaining tables.

Tungsten, as mentioned above, has commonly been considered in the prior art to be a potential substitute for molybdenum but not at the low carbon levels here concerned. In Table III below, an 8% tungsten addition as

50 a complete substitute for molybdenum (Alloy V) produces severe cracking, and in fact this heat was so weak that it could not even be tested for corrosion rates. A substitution of 4% tungsten for that same amount of molybdenum causes moderate cracking and lowers the 55 corrosion resistance of the material considerably. Even the straight addition of tungsten to the optimum alloy composition, as in Alloy N, causes loss of corrosion resistance.

Table III

| Alloy | Percent Mo | Percent W | Hardness |    | Mean Corrosion Rate, Mils Per Year 5-48 Hour Test Periods |                |                |                  |                  |                  |
|-------|------------|-----------|----------|----|-----------------------------------------------------------|----------------|----------------|------------------|------------------|------------------|
|       |            |           | BHN      | Rc | 65 N,<br>Boil.                                            | 10 S,<br>Boil. | 30 S,<br>Boil. | 70 S,<br>176° F. | 15 H,<br>125° F. | 20 H,<br>100° F. |
| A     | 8.0        | Nil       | 270      | 28 | 8                                                         | 11             | 114            | 14               | Nil              | 35               |
| U     | 4.0        | 4.0       | 234      | 22 | 11                                                        | 24             | 314            | 75               | 145              | 67               |
| V     | Nil        | 8.0       | 238      | 21 | 8                                                         | 11             | 210            | -----            | Nil              | 50               |
| N     | 8.0        | 3.0       | 276      | 29 | -----                                                     | -----          | -----          | -----            | -----            | -----            |

\*Samples could not be cut without cracking severely.

Like molybdenum, chromium contributes to both hardness and corrosion resistance. Corrosion rates of alloys at different levels of chromium are shown in Table IV. Optimum conditions for corrosion resistance are provided in alloys containing between 27 and 30% chromium. Up to around 32% can be used under certain circumstances. But it will be noted that at 35% chromium the corrosion resistance has depreciated considerably. Similarly, around 26% to 27% represents a lower limit from the standpoint of adequate hardness.

Table IV

| Alloy  | Percent Cr | Hardness |    | Mean Corrosion Rate, Mils Per Year 5-48 Hour Test Periods |                |                |                  |                  |                  |
|--------|------------|----------|----|-----------------------------------------------------------|----------------|----------------|------------------|------------------|------------------|
|        |            | BHN      | Rc | 65 N.<br>Boil.                                            | 10 S.<br>Boil. | 30 S.<br>Boil. | 70 S.<br>175° F. | 15 H.<br>125° F. | 20 H.<br>100° F. |
| Z----- | 23.0       | 255      | 25 | 14                                                        | 17             | 136            | 28               | 72               | 50               |
| A----- | 27.0       | 270      | 28 | 8                                                         | 11             | 114            | 14               | Nil              | 35               |
| J----- | 30.0       | 276      | 29 | 7                                                         | 9              | 159            | 29               | 30               | 80               |
| D----- | 35.0       | 382      | 41 | 20                                                        | 30             | 359            | 30               | 476              | 182              |

The amount of nickel in the alloy composition up to and including 10% does not significantly change the corrosion resistance of the alloys to various mineral acids such as nitric, sulfuric and hydrochloric. Best over-all results occur at about 2% nickel, and this is accordingly a preferred level. However, the hardness of the alloys drops off sharply with increase in nickel content, and at 10% nickel this becomes approximately 200 BHN for the low molybdenum level alloys. By increasing the molybdenum content it is possible however to meet the desired BHN level even with 10% nickel, especially with work hardening, as by shot peening.

Corrosion rates in various media and hardness values for different levels of nickel content are shown in Table V.

Table V

| Alloy  | Percent Ni | Hardness |     | Mean Corrosion Rate, Mils Per Year 5-48 Hour Test Periods |                |                |                  |                  |                  |
|--------|------------|----------|-----|-----------------------------------------------------------|----------------|----------------|------------------|------------------|------------------|
|        |            | BHN      | Rc  | 65 N.<br>Boil.                                            | 10 S.<br>Boil. | 30 S.<br>Boil. | 70 S.<br>175° F. | 15 H.<br>125° F. | 20 H.<br>100° F. |
| O----- | Nil        | 290      | 31  | 14                                                        | 6              | 200            | 38               | 60               | 66               |
| A----- | 2.0        | 270      | 28  | 8                                                         | 11             | 114            | 14               | Nil              | 35               |
| P----- | 4.0        | 260      | 24  | 11                                                        | 6              | 152            | 36               | Nil              | 72               |
| Q----- | 6.5        | 255      | 23  | 10                                                        | 8              | 140            | 18               | 16               | 65               |
| E----- | 10.0       | 195      | *92 | 10                                                        | 9              | 120            | 25               | 40               | 43               |

\*This value is recorded as Rockwell "B."

Copper additions up to 4.5% do not noticeably affect the corrosion resistance except in medium and concentrated sulfuric acid and in this corrosive a level of 1.75 to 4.5% appears to provide good results, as seen in Table VI. Acceptable results for many uses are still obtainable at a low of 1.5% copper. Corrosion resistance to medium concentrations of sulfuric acid suffers considerably as the copper content falls substantially below 1.5% or goes above 4.5%, as shown by Alloys R and T. Hardness of the alloys is slightly increased by removing all of the copper, but the slight benefit to hardness is more than offset by the decreased corrosion resistance.

As already pointed out, the carbon level is critical. When increased quantities of chromium and molybdenum are employed in the presence of carbon much above 0.10%, hardness is increased but corrosion resistance is seriously lowered, especially in oxidizing media. Additions of up to 0.10% carbon, or slightly more, have no appreciable effect on corrosion resistance of the relatively ductile alloys (e.g. Alloy A), provided they are properly heat treated; however, an addition of 0.20% carbon reduces the corrosion resistance of all invention alloys in

almost all media. Since the harder compositions within the invention cannot be adequately heat treated to eliminate corrosion-producing carbide formation, at least not without danger of so straining the material as to cause cracking to occur, carbon levels in the harder compositions of the type used for shaft sleeves should be held to a maximum of 0.03%.

It is also quite apparent that as the molybdenum content of the alloy is increased it is necessary to decrease proportionately the tolerable amount of carbon in order to obtain a given degree of corrosion resistance. The susceptibility to formation of complex carbides containing molybdenum, and probably chromium also, increases as the molybdenum content itself increases, and since such

carbide formation adversely affects corrosion resistance, proper control of carbon is essential. It may be noted that the use of strong carbide formers such as columbium to preferentially tie up excess carbon is a definite possibility. This must be balanced in turn against deterioration in corrosion resistance if too much columbium is added. In other words, in all cases the molybdenum-plus-chromium to carbon relationship must be adjusted for each alloy composition within the specified molybdenum and chromium ranges to achieve the desired hardness and corrosion resistance.

60 Table VII compares the corrosion resistance of what

Table VI

| Alloy  | Percent Cu | Hardness |    | Mean Corrosion Rate, Mils Per Year 5-48 Hour Test Periods |                |                |                  |                  |                  |
|--------|------------|----------|----|-----------------------------------------------------------|----------------|----------------|------------------|------------------|------------------|
|        |            | BHN      | Rc | 65 N.<br>Boil.                                            | 10 S.<br>Boil. | 30 S.<br>Boil. | 70 S.<br>175° F. | 15 H.<br>125° F. | 20 H.<br>100° F. |
| R----- | Nil        | 305      | 32 | 8                                                         | 11             | 238            | 123              | Nil              | 44               |
| S----- | 1.75       | 285      | 30 | 8                                                         | 12             | 103            | 25               | Nil              | 49               |
| A----- | 3.25       | 270      | 28 | 8                                                         | 11             | 114            | 14               | Nil              | 35               |
| G----- | 4.5        | 285      | 24 | 6                                                         | 8              | 83             | 22               | Nil              | 61               |
| T----- | 5.0        | 278      | 29 | 9                                                         | 12             | 171            | 53               | 143              | 69               |

may be termed the normal carbon (0.06%) and low carbon (0.025%) alloys, as well as the effect at higher carbon contents.

used only for the milder applications. The effect of the addition of elements like aluminum and titanium on the hardness of typical alloys within the invention range is

Table VII

| Alloy | Percent C | Hardness |    | Mean Corrosion Rate, Mils Per Year 5-48 Hour Test Periods |             |             |              |               |               |
|-------|-----------|----------|----|-----------------------------------------------------------|-------------|-------------|--------------|---------------|---------------|
|       |           | BHN      | Re | 65 N, Boil.                                               | 10 S, Boil. | 30 S, Boil. | 70 S, 80° C. | 15 H, 125° F. | 20 H, 100° F. |
| M     | .025      | 376      | 40 | 12                                                        | 12          | 130         | 20           | Nil           | 35            |
| K     | .06       | 375      | 40 | 35                                                        | 10          | 130         | 27           | Nil           | 40            |
| A     | .07       | 270      | 28 | 8                                                         | 11          | 114         | 14           | Nil           | 35            |
| X     | .10       | 265      | 27 | 10                                                        | 5           | 81          | 25           | Nil           | 35            |
| W     | .20       | 270      | 28 | 35                                                        | 7           | 153         | 25           | 20            | 20            |

The addition of iron to the novel alloys produces progressive loss in corrosion resistance, although the change is primarily significant only in the more severe media. For best resistance a maximum of 6% iron has been found to be a desirable upper level to be observed and again this may be resorted to for increased hardness in the alloy if the accompanying loss in corrosion resistance can be tolerated or can be compensated for by further adjustment of other elements, e.g. nickel. Table VIII gives examples of relative corrosion resistance at various iron levels.

20 shown in Table X.

Table X

| Treatment                               | Hardness, BHN |         |         |
|-----------------------------------------|---------------|---------|---------|
|                                         | Alloy A       | Alloy H | Alloy I |
| As Cast                                 | 265           | 265     | 265     |
| Anneal 2 hrs. at 2250° F., water quench | 270           | 275     | 240     |
| Anneal 6 hrs. at 1200° F., air cool     | 265           | 265     | 265     |
| Anneal 6 hrs. at 1400° F., air cool     | 276           | 297     | 290     |
| Anneal 6 hrs. at 1600° F., air cool     | 265           | 332     | 210     |
| Anneal 6 hrs. at 1800° F., air cool     | 260           | 370     | 350     |

Table VIII

| Alloy | Percent Fe | Hardness |    | Mean Corrosion Rate, Mils Per Year 5-48 Hour Test Periods |             |             |              |               |               |
|-------|------------|----------|----|-----------------------------------------------------------|-------------|-------------|--------------|---------------|---------------|
|       |            | BHN      | Re | 65 N, Boil.                                               | 10 S, Boil. | 30 S, Boil. | 70 S, 80° C. | 15 H, 125° F. | 20 H, 100° F. |
| A     | 2          | 270      | 28 | 8                                                         | 11          | 114         | 14           | Nil           | 35            |
| DD    | 6          | 276      | 29 | 8                                                         | 8           | 151         | 22           | Nil           | 56            |
| EE    | 10         | 290      | 30 | 8                                                         | 19          | 223         | 22           | Nil           | 81            |

Additional modifiers which are normally included are silicon and manganese, both in amounts not exceeding approximately 2%, and generally each is preferably at levels below 1%, especially in the case of silicon. In the case of silicon (see Table IX), additions of 1.5% to 3% increase the BHN, but corrosion resistance of the resulting alloys is adversely affected, especially under the more severe service conditions. Low silicon levels of 0.3% have been maintained successfully in casting small cross sections and present indications are that silicon is not needed for fluidity in the alloys.

45 Aluminum and titanium do not influence the alloy microstructure in the as-cast condition or when the alloys are quench annealed from approximately 2250° F. But these additions do have a definite effect when the resulting alloys are annealed at temperatures within the range of 1400° F. to 1800° F. Hardening is influenced by the formation of sigma phase in the standard or normal (0.06%) carbon alloy. Diffusion rates of chromium and other elements are slow in the presence of cobalt, and even annealing the base composition (Alloy A) at 1800° F. for 6 hours will cause very little sigma phase to form.

Table IX

| Alloy | Percent Si | Hardness |    | Mean Corrosion Rate, Mils Per Year 5-48 Hour Test Periods |             |             |              |               |               |
|-------|------------|----------|----|-----------------------------------------------------------|-------------|-------------|--------------|---------------|---------------|
|       |            | BHN      | Re | 65 N, Boil.                                               | 10 S, Boil. | 30 S, Boil. | 70 S, 80° C. | 15 H, 125° F. | 20 H, 100° F. |
| A     | 0.5        | 270      | 28 | 8                                                         | 11          | 114         | 14           | Nil           | 35            |
| BB    | 1.5        | 322      | 34 | 9                                                         | 13          | 148         | 22           | Nil           | 66            |
| CC    | 3.0        | 302      | 39 | 43                                                        | 30          | 388         | 33           | 93            | 182           |

Manganese in small percentages up to 2% may be used for deoxidizing and hardening. Other deoxidants such as calcium may be employed. Also, small additions of other hardening agents such as aluminum and titanium can be employed. In general such additions are kept low, not in excess of about 1% each, and preferably below this. Boron is also a good hardening agent but since it has a deleterious effect on corrosion resistance, it may be

70 In fact it requires about 16 hours to cause a significant change in hardness in such alloy. The addition of small amounts of aluminum and titanium, however, results in large quantities of sigma phase being formed (see Alloys H and I of Table X) in relatively short times.

75 The shaft sleeve alloy (e.g. Alloy M) shows a tendency to increase in hardness in the 1400° to 1800° F. range, probably because of the observed greater amount of

secondary phase which accompanies this treatment. It is this secondary phase in the microstructure which accounts for varied hardness.

The effects of heat treatment and cold working of the alloys of the invention are important to their corrosion resistance. Quenching from temperatures as high as 2250° F. does not affect their original hardness; however, alloys of the harder composition (e.g. shaft sleeve Alloy M) may tend to crack because of lower thermal shock resistance if a severe quench, such as water, is used. Therefore, it is generally recommended that these harder compositions normally be air cooled from the elevated temperature. Such air cooling has proved to be sufficiently rapid to maintain the same corrosion resistance as obtained from water quenching.

Cold working the harder alloys rapidly lowers their corrosion resistance, even when a relatively mild amount of working, such as shot peening, is used. The more ductile compositions, however, are not appreciably affected in corrosion resistance by shot peening although more severe deformation, e.g. a 5% reduction of area, produces very serious changes, particularly in respect to lowered resistance in hydrochloric acid. As mentioned, work hardening of the softer alloys (e.g. 270 BHN) provides an important method of increasing their usefulness.

There appears, on first glance, to be a general similarity in chemical composition between alloys of this invention and others in the prior art. However the specific differences and refinements introduced by the present teaching result in very decided differences in corrosion resistance and hardness, which are unique and are not merely a matter of degree. It may be significant to point out in this connection that the teaching of the prior art in respect to obtaining increased hardness in the prior alloys is generally by way of promoting the formation of various carbides through addition of strong carbide formers in the presence of adequate carbon to permit this. This however adversely affects corrosion resistance. The discovery of the particular combination of alloying elements herein defined, on the other hand, provides a way of increasing hardness by the formation of other hard, intermetallic compounds without sacrificing corrosion resistance. This is accomplished by carefully controlling the composition of the alloys as described above.

What is claimed is:

1. A cast cobalt base alloy having substantially the following composition:

|    | Percent by weight                         | 50 |
|----|-------------------------------------------|----|
| Cr | 30.                                       |    |
| Mo | 13.                                       |    |
| C  | 0.03 max.                                 |    |
| Cu | 3.25.                                     |    |
| Mn | 0.5.                                      |    |
| Si | 0.5.                                      |    |
| Fe | 2.0.                                      |    |
| Ni | 2.0.                                      |    |
| Co | Balance except for incidental impurities. |    |

2. A cast cobalt base alloy as defined in claim 1, wherein said alloy has a Brinell of about 375.

3. A cast cobalt base alloy having substantially the following composition:

|       | Percent by weight                         |
|-------|-------------------------------------------|
| Cr    | 28.                                       |
| Mo    | 8.5.                                      |
| C     | 0.10 max.                                 |
| 10 Cu | 3.25.                                     |
| Mn    | 0.5.                                      |
| Si    | 0.5.                                      |
| Fe    | 2.0.                                      |
| Ni    | 2.0 to 10.0.                              |
| 15 Co | Balance except for incidental impurities. |

4. A corrosion and abrasion resistant alloy as defined in claim 3, wherein the alloy has a Brinell of at least 270.

5. A corrosion and abrasion resistant alloy as defined in claim 3, wherein the alloy has a Brinell of at least 300.

6. A corrosion and abrasion resistant cobalt base alloy containing by weight from approximately 26% to 32% chromium, from 8% to 15% molybdenum, not exceeding about 0.10% carbon, from 1.5% to 4.5% copper, up to 10% nickel, up to 6% iron and conventional hardening, deoxidizing and carbon stabilizing modifiers which aggregate not more than about 3%, the balance being substantially all cobalt except for incidental impurities, said alloy having its carbon content adjusted within the stated range in accordance with the chromium-molybdenum content to maintain an as-cast hardness of at least about 270 Brinell, the carbon being below about 0.03% at the higher levels of molybdenum and chromium to compensate for the increased tendency toward carbide formation and accompanying decreased corrosion resistance.

#### References Cited by the Examiner

##### UNITED STATES PATENTS

|           |       |                  |          |
|-----------|-------|------------------|----------|
| 1,528,478 | 3/25  | Hadfield         | 75-171   |
| 1,807,554 | 5/31  | Rohn             | 75-171   |
| 2,072,910 | 3/37  | Touceda          | 75-171   |
| 2,072,911 | 3/37  | Touceda          | 75-171   |
| 2,081,392 | 5/37  | Touceda          | 75-171 X |
| 2,180,549 | 11/39 | Prange           | 75-171 X |
| 2,309,136 | 1/43  | Neiman           | 75-171   |
| 2,403,128 | 8/46  | Scott et al.     | 75-171   |
| 2,419,825 | 4/47  | Dinerstein       | 75-171   |
| 2,524,661 | 10/50 | Harder et al.    | 75-171   |
| 2,631,095 | 3/53  | Griffiths et al. | 75-171   |
| 2,761,778 | 9/56  | Mann             | 75-171   |
| 2,777,766 | 1/57  | Binder           | 75-171   |

DAVID L. RECK, Primary Examiner.

UNITED STATES PATENT OFFICE  
CERTIFICATE OF CORRECTION

Patent No. 3,177,074

April 6, 1965

Walter A. Luce et al.

It is hereby certified that error appears in the above numbered patent requiring correction and that the said Letters Patent should read as corrected below.

Column 1, line 22, for "acid" read -- acids --; line 42, for "noval" read -- novel --; column 4, lines 27 and 31, for "dutility", each occurrence, read -- ductility --; column 5, Table I, in the footnote, line 5 thereof, for "test" read -- text --; column 8, line 26, for "wthin" read -- within --; column 10, Table X, fourth column, line 5 thereof, for "210" read -- 310 --.

Signed and sealed this 21st day of September 1965.

(SEAL)

Attest:

ERNEST W. SWIDER  
Attesting Officer

EDWARD J. BRENNER  
Commissioner of Patents